

# UNITED STATES PATENT OFFICE.

WILLIAM HOSKINS, OF CHICAGO, ILLINOIS.

## ART OF RECOVERING POTASH.

1,307,127.

Specification of Letters Patent. Patented June 17, 1919.

No Drawing.

Application filed January 12, 1917. Serial No. 142,099.

To all whom it may concern:

Be it known that I, WILLIAM HOSKINS, a citizen of the United States, residing at Chicago, in the county of Cook and State of Illinois, have invented a new and useful Improvement in the Art of Recovering Potash, of which the following is a specification.

My invention relates to the art of recovering potassium and its compounds and will 10 be fully understood from the following specification.

In brief, I have discovered that the ordinary grades of coal used for fuel in industrial furnaces and the like, and such, for instance, as Illinois and Indiana bituminous coal, may, under certain conditions, form a 15 technically useful and valuable source of supply for potassium and its compounds.

Although, in view of the commercial importance of the matter, and of the deep study and widespread prevalent knowledge of the 20 chemical composition of coal, it may have been previously known that coal contains traces of potassium as well as traces of most 25 of the common elements native to the soil or to the various sub-surface strata of the locality in which the coal occurs, such traces of an exceedingly large number of elements, appearing from a spectrum analysis of al- 30 most any sample of coal, it is certain that the presence of potassium was either wholly unknown or was regarded as entirely negligible. An examination of the writings of the recognized authorities on the subject dem- 35 onstrates that if potassium had, in fact, been discovered in coal, it was completely ignored in the statements of analysis.

So also the ash, or residue, resulting from 40 the combustion of coal of every common variety has been repeatedly subjected to the most careful study, but here, also, there is no indication that anything more than quantitatively undeterminable traces of potassium could be found.

45 I have discovered, however, that the ordinary grades of coal referred to, when burned in the usual manner in the furnaces of boilers, form a technically valuable source of supply of potassium. The minute quantities or traces of potassium present in the native coal are volatilized by the heat of combustion, and are carried out of the combustion chamber along with a relatively small 50 proportion of unburned carbon, ash, and small quantities of other substances.

This matter, which is either solid, or condensable, and which continuously passes out of the combustion chamber, is relatively small in proportion to the mass of coal burned, but in the aggregate amounts to a 60 very considerable quantity, especially in large industrial establishments, such, for instance, as public service electric light and power generating stations. The solid and condensable matter carried out of the combustion chamber of the furnace collects or 65 deposits, in the first instance, immediately behind the bridge wall, or in the breeching or equivalent structure of the furnace, accumulating in the form of a friable slag which 70 is periodically broken up and cleaned out by the furnace attendants. A certain further proportion of the solid or condensable constituents carried along by the combustion gases escape deposition at this place, how- 75 ever, and is caught as soot on the walls of the economizers, flues, stacks or other surfaces over which the combustion gases pass before being vented to the atmosphere.

The slag and soot deposited from the outgoing combustion gases in the manner described, I find to contain workable quantities of potassium or its compounds. Apparently, the process of combustion as ordinarily carried out in the manner above de- 80 scribed, automatically affects the concentration of whatever potassium may have been present in the original coal, and this concentration process is so effective that quantities of potassium, so minute as to be quantita- 85 tively undeterminable in the original coal, appear as workable percentages in the slag and soot "concentrate."

For example, it is found that a certain 90 industrial establishment burns in the neighbor- 95 hood of 96,000 tons of coal per month, producing in that period 900 tons of slag and 55 tons of soot. By analysis these "concentrates" are found to contain the following proportion of potassium (figured as 100 K<sub>2</sub>O):

|      |       |       |
|------|-------|-------|
| Slag | ----- | .60%  |
| Soot | ----- | 1.75% |

Of this quantity of potash approximately 105 75% may be recovered by merely leaching with warm or hot water. The total recovery of potash from the plant in question would, therefore, be of the order of 5½ tons per month.

The foregoing example is representative of the quantities of soot obtainable in the ordinary industrial establishment. It is, of course, quite possible to employ soot collecting or dust collecting methods or means by which the quantity of soot recoverable from the combustion gases may be largely increased.

It therefore appears that by the ordinary process of combustion as carried out in industrial furnaces, the minute quantities or traces of potassium in the native coal become automatically concentrated in the solid or condensable matter deposited by the combustion gases, the concentration proceeding so far as to afford a source of potassium which may be technically utilized by the simple expedient of leaching, the resultant potash solution being evaporated to dryness by waste heat from the furnaces which produce the raw material, or the potash being recovered in any other appropriate manner. In view of the fact that the industrial furnaces of this country continuously consume hundreds of millions of tons of coal in each year, such coal consumption, according to the ordinary methods, necessarily resulting in the formation of a potassium "concen-

trate" containing workable quantities of potash, it will be understood that my invention affords a new source of supply for the element in question of noteworthy technical importance.

What I claim as new and desire to secure by Letters Patent is:

1. The method of obtaining potash, which consists in collecting the solid and condensable matter carried by the gases resulting from the combustion of coal in industrial furnaces, and extracting the potash from the said solid matter.

2. The method of obtaining potash, which consists in collecting the solid and condensable matter carried by the gases resulting from the combustion of coal in industrial furnaces, and leaching out the potash from said solid matter.

3. The method of obtaining potash, which consists in collecting the solid and condensable matter carried by the gases resulting from the combustion of coal in industrial furnaces, leaching out the potash from said solid matter, and evaporating the potash solution thus obtained by the heat resulting from the combination of the said coal.

WILLIAM HOSKINS.

Copies of this patent may be obtained for five cents each, by addressing the "Commissioner of Patents, Washington, D. C."